

Patented Dec. 18, 1928.

1,695,430

# UNITED STATES PATENT OFFICE.

JAMES D. KLINGER, OF DETROIT, MICHIGAN.

AGENT FOR CLEANING AND IMPARTING RUST-INHIBITIVE PROPERTIES TO STEEL.

No Drawing.

Application filed June 27, 1924. Serial No. 722,720.

My invention relates to an improved method of cleaning and preparing steel for painting. The object is to provide an improved method and agent through the use 5 of which steel may be cleaned and rust resisting properties imparted hereto.

This invention is particularly valuable in connection with the preparation of the sheet steel employed in the manufacture of automobile bodies. The grease, dirt, oil, rust, etc., must be cleaned from this sheet steel and the surface prepared to receive the priming coat of paint. To meet this commercial demand, it is essential that the method, and agent employed therein, be inexpensive, and that the process be a rapid one. By following my improved process the steel is thoroughly cleaned so as to receive and retain the priming coat of paint and the surface of the metal 20 is rendered substantially immune to the subsequent action of rust.

I provide a suitable cleaning solution which is applied as a wash or a bath to the metal to be treated to remove the grease, oil, dirt, 25 rust, etc. For this purpose I prefer to employ a solution composed of an effective rust attacking and removing acid, such as sulfuric acid, and a solvent for the oil, grease, etc., such as alcohol or acetone. Denatured alcohol containing a small percentage of acetone 30 makes a very satisfactory solvent.

I have found that by using a cleaning solution such as above containing as an added ingredient, a suitable hydroxycarboxylic acid, that rust inhibitive properties will be imparted to the surface of the metal. The hydroxycarboxylic acid in the solution acts upon the metal and prevents the formation of iron hydroxide, which is the first stage of rust, and 40 which otherwise would occur as a result of the presence of the sulfuric acid and the water. I prefer to employ in this connection a hydroxytricarboxylic acid, of which the most common one is citric acid. However, hydroxydicarboxylic acid, such as tartaric acid 45 is effective for the purpose.

Generally stated, this invention consists in applying a fluid admixture of a hydroxycarboxylic acid, a rust attacking and removing acid and a solvent for oil and grease to the steel to be treated, which solution removes all oil, grease, dirt, rust, etc., from the surface of the material and gives it a bright, clean finish, prevents the formation of iron hydroxide thereon, and imparts rust resisting properties thereto.

The cleaning solution may be applied to the metal by painting or spraying the metal therewith. A period from two to three minutes should be allowed for the solution to act. 60 In cases where there is deep-seated rust on the steel the cleaning solution and the resultant products of the cleaning action are washed from the steel by rinsing with hot or cold water. If cold water is used, it should 65 be flowed on freely and the water remaining on the steel blown off with air. If hot water is used any water that has not evaporated should be blown off with air. The water should be completely removed from the surface of the metal and it may be necessary to torch off around mouldings or pockets with a gas flame to drive out the remaining water. The steel should then be wiped with a cloth 70 saturated with turpentine or alcohol and placed in a pre-heat oven to dry. The steel 75 is now ready to receive the priming coat of paint.

The strength of the solution and the proportion of the respective ingredients may be 80 varied to meet the exigencies of the material to be cleaned. I have found, however, that a solution comprising sulfuric acid, citric acid and denatured alcohol having a small percentage of acetone is particularly effective, 85 and a very satisfactory strength is to provide these ingredients in the proportion, by volume, of thirty-five parts of an aqueous solution of citric acid (strength of solution twenty per cent), five parts of concentrated sulfuric acid, fifty parts of denatured alcohol 90 and ten parts of acetone.

What I claim is:

1. A solution to be used in the cleaning of steel and the imparting of rust inhibitive properties thereto containing the following ingredients in substantially the approximate volume of five parts of alcohol, four parts of citric acid and one part of sulfuric acid. 95
2. A solution to be used in the cleaning of steel and the imparting of rust inhibitive properties thereto containing the following ingredients in substantially the approximate volume of five parts of alcohol, and five parts of citric acid, sulfuric acid and acetone, with 100 citric acid predominating.
3. A solution to be used for cleaning and imparting rust resisting properties to steel containing a solvent for grease and oil, a rust removing acid and a hydroxycarboxylic acid. 110
4. A solution to be used for cleaning and

imparting rust resisting properties to steel containing denatured alcohol, an aqueous solution of citric acid, sulfuric acid and a small percentage of acetone.

5. A solution to be used for cleaning and imparting rust resisting properties to steel containing a hydroxycarboxylic acid.

6. A solution to be used for cleaning and imparting rust resisting properties to steel containing a hydroxytricarboxylic acid.

In testimony whereof, I sign this specification.

**JAMES D. KLINGER.**